

Nov. 5, 1968

R. J. LOKKEN

3,409,438

PHOTOSENSITIVE HEAT DEVELOPABLE COPYSHEET

Filed Aug. 26, 1963

3 Sheets-Sheet 1

FIG. 1



FIG. 2



FIG. 3



FIG. 4



FIG. 5



FIG. 6



FIG. 7



FIG. 8



FIG. 9



FIG. 10



FIG. 11



FIG. 12



FIG. 13



FIG. 14



FIG. 15



FIG. 16



FIG. 17



FIG. 18



FIG. 19



INVENTOR

ROBERT J. LOKKEN  
BY

Carpenter, Abbott, Coulter & Kinney  
ATTORNEYS

Nov. 5, 1968

R. J. LOKKEN

3,409,438

PHOTOSENSITIVE HEAT DEVELOPABLE COPSHEET

Filed Aug. 26, 1963

3 Sheets-Sheet 2

FIG. 20



FIG. 21



FIG. 22



FIG. 23



FIG. 24



FIG. 25



FIG. 26



INVENTOR.

ROBERT J. LOKKEN  
BY

Carpenter, Abbott, Coulter & Kinney  
ATTORNEYS

Nov. 5, 1968

R. J. LOKKEN

3,409,438

PHOTOSENSITIVE HEAT DEVELOPABLE COPIYSHEET

Filed Aug. 26, 1963

3 Sheets-Sheet 3

FIG. 27



FIG. 28



FIG. 29



FIG. 30



FIG. 31



FIG. 32



FIG. 33



FIG. 34



FIG. 35



FIG. 36



FIG. 37



FIG. 38



FIG. 39



FIG. 40



FIG. 41



INVENTOR

ROBERT J. LOKKEN  
BY

Carpenter, Abbott, Coulter & Kinney  
ATTORNEYS

1

3,409,438  
**PHOTORESITIVE HEAT DEVELOPABLE  
COPYSHEET**

Robert J. Lokken, Maplewood, Minn., assignor to Minnesota Mining and Manufacturing Company, St. Paul, Minn., a corporation of Delaware

Filed Aug. 26, 1963, Ser. No. 304,422  
19 Claims. (Cl. 96—95)

## ABSTRACT OF THE DISCLOSURE

A light-sensitive copysheet, which develops an intense silver image by simple heating after exposure, contains a water-insoluble silver soap of a fatty acid together with a light-sensitive progenitor of a reducing agent for silver ion.

This invention relates to copysheet products which after exposure to actinic radiation are visibly sensitive to heat.

Copysheets prepared in accordance with the invention have particular utility in making positive prints from photographic negatives.

Photographic processes based on photosensitive silver halide coatings normally produce negative transparencies in which the darks and lights of the subject photographed are transposed. A second transposal is therefore required in order to obtain a true reproduction of the original subject. In traditional photographic processes this involves exposure, through the negative transparency, of a silver halide print paper which must then be subjected to a wet developing process in order to bring out the desired positive visible image. The present invention provides a dry process printing paper on which the positive or transposed image is obtained by a simplified process involving merely exposure to the negative light-image followed by uniform mild heating of the exposed sheet.

In an alternative procedure the sensitive copysheet is first uniformly exposed to actinic radiation to render it visibly sensitive to heat, after which it is used to provide a permanent visible record of a heat-image impressed thereon, e.g. by means of a heated stylus or heated metal type, or by thermographic copying processes, or in other ways.

Heat-sensitive copysheets having particular utility in the reproduction of graphic originals by thermographic copying processes have previously been known. As described in Owen U.S. Patent No. 2,910,377, one useful form of heat-sensitive composition contains a silver soap and a reducing agent. A typical formulation includes silver behenate and a polyhydroxyaromatic reducing agent such as dihydroxybenzoic acid, together with suitable stabilizers, toners, polymeric binders and other modifiers as desired. These copysheets are essentially stable toward light and are permanently visibly changed from white to intense blue-black on momentary heating to temperatures in the range of about 90—150° C. In Grant U.S. Patent No. 3,904,619, the selection of certain specific types of hydroxyaromatic reducing agents permits these heat-sensitive silver soap compositions to be desensitized by exposure to ultraviolet radiation, thereby permitting the formation of heat-stable black-on-white copies of black-on-white originals. The introduction of photoreducible dyes, as described in Workman U.S. Patent No. 3,094,417, permits the same results to be attained on exposure to visible light.

The preparation of positive or black-on-white copies by transposal from negative or white-on-black transparency originals in accordance with the present invention likewise involves the reduction of a silver salt to yield the silver image. However, unlike those of prior art copysheets, the sensitive coating initially contains no reducing

2

agent for the silver ion, or at most contains no reducing agent operable by itself at the temperature and within the time employed to cause reduction of the silver ion. Instead it contains a photosensitive silver reductant progenitor, i.e., a material which on irradiation undergoes a photochemical reaction with generation of a reducing agent for silver ion. The coated sheet accordingly is heat-resistant as initially produced, but is rendered heat-sensitive by exposure to actinic radiation, particularly to radiation in the near-ultraviolet range of wavelengths.

After exposure to a light-image and development of the visible image by heating, many of the copysheets of this invention may be exposed to normal room light for prolonged periods without visible change and without becoming heat-sensitive at unprinted background areas. Exposure to more intense radiation, particularly in the near-ultraviolet range, sensitizes these areas so that additional images may be formed by appropriate application of heat. In some instances the sheet may be desensitized by heating, e.g., by the removal of unused portions of the photosensitive silver reductant progenitor either by decomposition or by volatilization, thus stabilizing the background areas against further sensitization and reaction. Copy prepared with these preferred copysheets is therefore stable against both actinic radiation and heat.

The copysheet may be illustratively represented by the following symbolic cross-sectional diagram:

Mixture of silver salt and photosensitive progenitor of a silver reducing agent  
Paper-like backing

Silver behenate is a preferred silver salt and its preparation in the form of an intimate blend of equal molar proportions of coprecipitated salt and behenic acid has been described, e.g., in the Owen patent. The salt may be prepared essentially free of the acid by proper proportioning of the reactants, and in this form is found to produce a somewhat more intense image in the copysheet; on the other hand, the presence of the added acid improves the water-resistance of the coating. Normally solid silver salts of other fatty acids, and particularly of the higher fatty acids, are also useful; silver stearate is a good example. Other fatty acids, e.g., stearic acid, and other water-resistant or waxy materials may analogously replace the behenic acid. However these components are not essential and may be omitted. Other normally solid silver salts may be used, as well as salts of other noble metals, for example gold stearate; but the silver soaps of long chain fatty acids are easily prepared, conveniently handled, relatively inexpensive, impart a high order of stability, and are preferred. In particular the silver soaps have been found to be stable against exposure to light, so that they may be prepared and processed under normal illumination.

With the silver salts it is desirable to use images toning materials so that maximum image density and color contrast may be attained. Phthalic anhydride is one such material; another and much preferred toner is phthalazinone. However a visible image may be obtained in the absence of these or analogous additives.

Polyhydroxyaromatic compounds, such for example as dihydroxybenzoic acid, methyl gallate, catechol, or 2,3-naphthalenediol, are known to be effective reducing agents for silver ion in heat-sensitive copysheet structures, cf. the Owen patent. The structure of certain photosensitive aromatic diazo compounds is such as to make their conversion to analogous polyhydroxy compounds, by hydrolytic photodecomposition, appear feasible. It has now been found that many such diazo compounds are indeed effective as photosensitive progenitors of reductants for

silver ion, while remaining unreactive with the silver salt in the absence of actinic radiation.

Other materials which have been found useful to at least a limited extent as photosensitive progenitors of reductants for silver ion include certain unsaturated carbonyl compounds, quinones, aryl esters of carboxylic acids, and styryl dye bases. In all instances the compound has an unsaturated aliphatic (or cycloaliphatic) structure, preferably containing at least one conjugate double bond system, or an aromatic ring having at least one substituent group with one or more double bonds or other unsaturation, and is absorptive of, and altered by, actinic radiation in the ultraviolet or visible region of the spectrum. At the same time, many closely similar compounds are found to be completely ineffective as reductant progenitors, or to be effective to such a limited extent that copiesheets prepared therewith are not practical. It has therefore been found impossible fully to define the useful classes of reactants by chemical structure. However, it has been found possible to distinguish the commercially useful materials from the inoperable or impractical products by means of a simple test procedure involving the irradiation of a dilute solution containing reactable quantities of both the proposed reagent and silver nitrate.

More specifically, a preferred test procedure involves dissolving about one-tenth gram of the proposed progenitor material in ten grams of a mixture of equal weights of ethanol and water, adding thereto about three grams of a saturated solution of silver nitrate in 95% ethanol, adjusting the acidity of the mixture to pH 5 to 6 by means of dilute nitric acid or ammonium hydroxide as required, and irradiating a two ml. portion in a Pyrex test tube for three minutes with the radiation from a B-H 6 high pressure mercury arc lamp at a distance of nine inches. In the event a precipitate forms during addition of the silver nitrate solution, it is removed by filtration and sufficient additional silver nitrate is added to insure the presence of unreacted silver nitrate prior to irradiation. Formation of a black silver precipitate in the solution or of a silver mirror on the glass tube, either during irradiation or after heating the irradiated solution for one-half hour at 60° C., indicates the compound tested to be an effective silver reductant progenitor. A control sample of the silver nitrate solution is similarly irradiated, heated, and examined; any change in the test sample must be appreciably greater than any appearing in the control sample in order to indicate an effective reactant.

The test as just described has provided strong positive results, in the form of an unmistakable silver precipitate or mirror deposit, with all reductant progenitor compounds which have been found to produce commercially acceptable intense images in copiesheets prepared from such compounds in conjunction with silver behenate. Compounds which are less effective in the copiesheet, producing faint or low-density images under optimum exposure to light and heat, may or may not give positive results in the solution test. A few compounds which are not visibly reactive under test conditions have produced faint or inadequate images when tested in copiesheet formulations, although in most instances such compounds are entirely ineffective in the copiesheet. In at least one specific instance, a compound giving positive test results has produced no visible image in the sheet form; the sheet product therefore failing to meet the requirements for the copiesheets of this invention, namely the ability to be made visibly heat-sensitive by exposure to actinic radiation.

The preparation of the dry process printing sheet ordinarily involves the application of one or more coatings of the silver salt and reducing-agent progenitor to a thin paper or film substrate or backing. Various binder materials are employed to retain the reactants in position and condition for reaction on the surface of the substrate. In larger proportions, a film-forming polymeric binder may itself serve as the carrier film; or the reactants may

be retained, e.g., in a porous fibrous backing, in the substantial absence of binder. Transparent paper or film backings permit the copy to be seen from either surface and are particularly useful in reflex copying procedures and for making copies which are to be used as projection transparencies; but opaque backings such as heavy paper or metal foil are also useful, providing the material used is adequately resistant to the temperatures required in the development of the visible image. The silver salt and reducing agent progenitor may if desired be applied to separate substrates; exposure of the progenitor coating to a suitable light-image, and heating the thus exposed sheet with the coated surface in contact with the silver-coated surface, then produces a visible reproduction of the exposed image areas on the latter. For this modification the reductant should be volatilizable and adequately stable so that it may be transferred in reactive condition to the silver-containing receptor sheet. Various other combinations and modifications are possible, as will be further indicated hereinafter.

The practice of the invention will now be further illustrated in terms of specific but nonlimiting examples, in which all proportions are given in parts by weight unless otherwise noted. In many of these examples there will be employed certain preferred coating compositions and coated sheet materials now to be described.

#### COMPOSITION I

|                                                        | Parts |
|--------------------------------------------------------|-------|
| 30 Equimolar blend of silver behenate and behenic acid | 2.88  |
| Zinc oxide                                             | 11.5  |
| Powdered terpene resin ("Piccolyte S-135")             | 2.30  |
| Silver image toner (phthalazinone)                     | 1.15  |
| 35 Stabilizer (tetrachlorophthalic anhydride)          | 0.05  |
| Polyvinyl acetate                                      | 1.75  |
| Cellulose acetate                                      | 2.88  |
| Volatile vehicle (acetone)                             | 77.5  |

The composition is applied to a heavy white paper backing with a coating knife or bar at an orifice of 3 mils to provide, after removal of volatile vehicle, a smooth uniform white coating weighing 1.2 grams per square foot, the coated sheet being here identified as Sheet I.

Another composition is produced by adding, to the formulation of Composition I, 0.5 part of a light-stable tertiary-alkyl phenol mild reducing agent, more specifically 2,6-di-tertiarybutyl 4-methylphenol, also known as "Ionol." The modified mixture is identified as Composition II and the corresponding coated sheet material as Sheet II. Where Sheet I remains white under prolonged exposure to moderately elevated temperatures of the order of 100° C., Sheet II under the same conditions will be found to darken slowly, becoming a dull brownish gray after several hours at that temperature or more rapidly at higher temperatures. However the reaction is not sufficiently rapid and the amount of the mild reductant is not sufficiently large to permit the copying of graphic originals on papers such as Sheet II on any practical basis by the thermographic process using commercially available thermographic copying machines.

#### Example 1

A first mixture consists of 48 parts of the equimolar blend of silver behenate and behenic acid dispersed in very small particles by prolonged ball milling in a solution of 12 parts of polystyrene (Dow 700) in a mixture of 152 parts of toluene, 102 parts of acetone and 84 parts of commercial heptane. To ten parts of the mixture thus prepared is added a solution of 0.25 part of phthalazinone in two parts of dioxane. The resulting composition is applied at a coating bar spacing of three mils to map overlay tracing paper, and the sheet is dried.

A second mixture is prepared by mixing together 0.2 part of potassium o-hydroxybenzenediazosulfonate, 0.2 part of sodium-1,3,6-naphthalenetrisulfonate, 0.2 part of

glycerine, 0.4 part of ethyl cellulose, six parts of acetone and one part of water. The second and third named ingredients are optional and may be omitted. The composition is coated at an orifice of three mils over the previous coat, and dried, these operations being conducted under subdued light.

The coated sheet is white in color. It is covered with a photographic negative transparency placed in contact with the coated surface and is exposed to light from a B-H 6 high pressure mercury arc ultraviolet lamp for ten seconds at a distance of eight inches. The exposed sheet remains visibly unchanged. It is then heated for one minute at 100° C. A visible transposed image is produced, having dense black image areas corresponding to the transparent portions of the negative, and a somewhat yellowish appearance at the remaining background areas.

The same compositions, applied to transparent Mylar film but in reverse order, produce a copysheet which when irradiated through the transparent film and heated as described results in a transposed copy showing significantly less discoloration at background areas.

#### Example 2

To the mixture identified as Composition I there is added 0.20 part of p-diethylaminobenzenediazonium hexafluorophosphate. The composition is coated on white paper and dried. The sheet is exposed through a transparency to light at about 8400 foot-candles as obtained from a light-box fitted with a number of tungsten filament lamps, exposure being for 15 seconds. The exposed sheet is then heated for eight seconds at 120° C. A sharp dense transposed copy of the transparency is obtained.

Equally effective results are obtained by substituting p-diethylaminobenzenediazonium tetrafluoroborate as the reductant progenitor.

The single coating is most conveniently applied, but suitable precautions must be taken to avoid exposure to light. Application of the reductant progenitor in a separate layer, as in Example 1, requires an additional process step but the silver coating may be compounded and applied in the light. An effective procedure involves the application of the diazonium fluophosphate or fluoroborate from solution by lightly uniformly swabbing the solution over the surface of the coating of Sheet I hereinbefore described. A typical solution for this purpose contains one part of the diazonium compound in five parts of ethanol and 94 parts of water.

#### Example 3

"Mylar" polyester film is coated at a 3 mil orifice with a composition consisting of two parts of methyl cellulose, 60 parts of methanol, 40 parts of water, and 1.25 parts of potassium o-hydroxybenzenediazosulfonate. The dry coating is exposed through a transparency to light at about 10,000 foot-candles from incandescent tungsten filament lamps for 15 seconds. The exposed film is then placed in face-to-face contact with a portion of Sheet II as hereinbefore described and the composite is heated between glass plates for about six seconds at 120° C. to provide on the Sheet II a transposed copy of the imaged transparency. The copy is removed and replaced with a second portion of Sheet II, and a second copy is produced by again heating the composite. A total of four copies is made, the time of heating being increased for each successive copy sufficiently to provide a corresponding image density in each instance and up to a final time of about 13 seconds, with essentially complete exhaustion of the reductant.

The addition to the coating composition of 0.1 part of erythrosin produces a pink-colored coated film which when similarly exposed through the transparency and heated against a succession of portions of Sheet II is found to yield a total of six copies before the reductant is exhausted, indicating that the presence of the photo-reducible dye initiates the conversion of increased amounts of the diazonium salt to a silver reducing agent.

Similar results are obtained using benzoquinone as the silver reductant progenitor and hematoporphyrin as the sensitizing photoreducible dye. The presence of the dye reduces the required exposure time and extends the spectral sensitivity toward the region of longer wavelength.

#### Example 4

A portion of Sheet II is further coated with a thin application of a one-half percent solution in methylethylketone of p-diethylaminobenzenediazonium hexafluorophosphate, as previously described in connection with Example 2. The dried sheet is exposed through a contacting photographic negative transparency to radiation from a carbon arc source, e.g., for about one-half minute, and is then heated at 130° C. for 7 seconds to produce a transposed copy having sharp and intense black image areas on a white background. In the absence of the diazonium compound the sheet yields no comparable image under the exposure and heating conditions specified, even though moderate irregular darkening occurs on extended heating, e.g., in one minute at 130° C.

#### Example 5

A one percent solution of thymoquinone in acetone is applied to a portion of Sheet I by means of a cotton swab. The sheet is dried, exposed to a light-image, and heated briefly at 100° C. to provide a transposed copy. Further heating at 100° C. removes the unreacted thymoquinone to stabilize the background areas against changes caused by further light-exposure without affecting the darkened image areas. Replacing the thymoquinone with 1,9-bis(2-furyl)-1,3,6,8-nonatetraene-5-one is equally effective. The compound phenanthrene quinone is similarly useful but a somewhat higher temperature of 125° C. is required. With 4,4'-bisdimethylaminobenzophenone a temperature of 135° C. is desirable. These silver reductant progenitor compounds are volatile at the temperatures indicated.

#### Example 6

A portion of Sheet II is lightly coated with a solution of 10 parts of phenyl chloroacetate and 15 parts of a copolymer of vinyl acetate and vinyl chloride (Vinylite VYHH) in 150 parts of acetone and 135 parts of toluene. The dried sheet is exposed through a negative for one-half minute to radiation from an AH-4 ultraviolet lamp. A positive print having dense black image areas is obtained on the coated sheet. During the exposure the temperature of the sheet does not exceed approximately 35-40° C. The images are not intensified by subsequent heating at higher temperatures. Where phenyl chloroacetate produces strong intense images, those produced by phenyl acetate are of medium intensity and by o-tolyl acetate are weak and indistinct. No image is produced on portions of the sheet coated with ethyl chloroacetate.

#### Example 7

A dilute solution of 1,9-bis(2-furyl)-1,3,6,8-nonatetraene-5-one in acetone is swabbed lightly and uniformly over the coated surface of a portion of Sheet I and dried. The yellowish coating is exposed through a transparency for 10 seconds to radiation from a B-H 6 lamp. The light image reaches the coating directly over one area, and at another area through a Corning CS 3-70 filter which limits the incident radiation to wavelengths greater than 4660 Angstroms. Brief heating of the sample produces a visible transposed image at the directly irradiated area but no visible change at the area irradiated through the filter.

The experiment is repeated but with the addition to the silver reductant progenitor solution of small amounts of each of the dyes eosin and Setoflavine T. The dried sheet has the color of burnt umber. The directly irradiated area produces a strong transposed image; the area irradiated through the filter yields a less dense but fully visible transposed image.

## Example 8

"Mylar" transparent polyester film is coated on one surface with a thin uniform layer of a mixture of 0.2 part of 4-methoxy-1-naphthol, 0.088 part of erythrosin, and 10 parts of ethyl cellulose, to provide a reddish light-transmissive sensitized intermediate film member as described in Workman U.S. Patent No. 3,094,417. The uncoated surface of the film is then coated with a mixture of benzoquinone and hematoporphyrin as described under Example 3. The doubly coated film is placed with the first coating in contact with a photographic negative backed up with a sheet of white light-reflective paper. Light at 8400 foot-candles from the light-box of Example 2 is directed through the film at the negative original for about one-half minute. The exposed film is then sandwiched between two portions of Sheet II and the composite is briefly heated in the range of about 100-130° C. by passing under moderate pressure around a heated roller. A copy of the transparency having the same light and dark areas is obtained on the sheet adjacent the first coating; a transposed copy is obtained on the sheet adjacent the second coating. The moderate darkening obtained at background areas of the transposed copy is eliminated by exposing through the negative rather than in the reflex position as described.

## Example 9

A transparent silver soap coating is provided on transparent Mylar polyester film using a composition containing 12 parts of silver behenate, 12 parts of polyethyl methacrylate, 1.8 parts of phthalazinone, 1.8 parts of 2,6-ditertiarybutyl-4-methylphenol, and 0.06 part of tetrachlorophthalic anhydride, applied in 44 parts of toluene and 132 parts of methylethylketone. The dry coating weighs 0.7 gram/sq. ft. Clarity is improved and the sheet is rendered light-sensitive by application of a further coating of 0.15 gram/sq. ft. of a mixture of 0.2 part of p-diethylaminobenzene diazonium tetrafluoroborate and 5 parts of cellulose acetate propionate applied as a 5% solution in methylethylketone. The sheet is exposed from the film side to light from the light-box of Example 2 for 15 seconds through a photographic negative. A portion of Sheet II is then placed in face-to-face contact with the exposed sheet and the composite is heated for seven seconds at 130° C. A transposed or positive copy of the negative original is produced on the Sheet II and also on the transparent film. In the latter, the areas corresponding to the opaque areas of the negative original remain clear and transparent, so that the product serves as an excellent projection transparency. At the same time the Sheet II positive copy is useful for inspection by the operator while the transparency is in the projector.

A list of photosensitive silver-ion-reductant progenitors which in conjunction with silver soaps have been found to provide light-activated heat-sensitivity in copysheets as herein described is here provided in tabular form, the corresponding structural formulas being indicated in the accompanying drawing.

| No. | Name                                                      |
|-----|-----------------------------------------------------------|
| 1   | potassium o-hydroxybenzenediazosulfonate                  |
| 2   | potassium p-hydroxybenzenediazosulfonate                  |
| 3   | potassium 2-hydroxy-5-chlorobenzene diazosulfonate        |
| 4   | potassium p-acetamidobenzene diazosulfonate               |
| 5   | sodium p-anilinobenzene diazosulfonate                    |
| 6   | potassium 2-hydroxy-3-chloro-5-nitrobenzenediazosulfonate |
| 7   | potassium 4-diethylamino-2-ethoxy-benzene diazosulfonate  |
| 8   | potassium 4-hydroxy-2-methylbenzenediazosulfonate         |
| 9   | 2-hydroxy-5-chlorobenzene diazo-p-toluenesulfonate        |
| 10  | di(p-anilinobenzene diazonium) sulfate                    |
| 11  | 1-diazo-2-naphthol-4-sulfonic acid                        |
| 12  | 4-diazo-1-naphthol-5-sulfonic acid                        |
| 13  | p-diethylaminobenzene diazonium tetrafluoroborate         |

- 14 p-dimethylaminobenzene diazonium tetrafluoroborate
- 15 4-diazo-N,N-diethyl-m-toluidine tetrafluoroborate
- 16 p-N,N-diethylaminobenzene diazonium hexafluorophosphate
- 17 stannous chloride salt of N-benzyl-N-ethylaniline-p-diazonium chloride
- 18 zinc chloride salt of 2-methyl-4-diethylaminobenzene-diazonium chloride
- 19 zinc chloride salt of N-ethyl-N-betahydroxyethylaniline-p-diazonium chloride
- 20 zinc chloride salt of 3-chloro-4-diethylaminobenzene-diazonium chloride
- 21 4,4'-bis-dimethylaminobenzophenone
- 22 4,4'-bis-dimethylaminothiobenzophenone
- 23 p-dimethylaminobenzalacetophenone
- 24 1,9-bis(2-furyl)-1,3,6,8-nonatetraene-5-one
- 25 1,5-bis(p-dimethylaminobenzal)-3-cinnamal-2,4-pentanediene
- 26 2,6-bis[3'-(2-furyl)acryl]cyclohexanone
- 27 p-benzoquinone
- 28 chloranil
- 29 thymoquinone
- 30 acenaphthenequinone
- 31 phenanthrene quinone
- 32 9-methyl-1,9-dihydro-2,6-naphthoquinone
- 33 1-chloroanthraquinone
- 34 phenyl chloroacetate
- 35 4-p-dimethylaminostyryl quinoline
- 36 2-p-dimethylaminostyryl quinoline
- 37 4,4'-dihydroxydiphenyltriazene

By way of comparison, the following structurally analogous compounds have been found ineffective as reductant progenitors in copysheets as here defined.

- 38 2-diazo-1-naphthol-5-sulfonic acid
- 39 p-nitrobenzenediazonium tetrafluoroborate
- 40 2,4-dinitrobenzenediazonium tetrafluoroborate
- 41 benzenesulfonic acid p-diazonium salt

40

## Example 10

It is possible with the sheet materials of this invention to produce a double transposition of image and background, thus for example making possible the preparation of a black-on-white copy from a black-on-white original. 45 One procedure involves making a first transposed copy e.g., by the procedure described in Example 1, irradiating the copy to convert the silver reductant progenitor to the reductant at the previously unexposed areas, and transferring the reductant to a reactive receptor sheet by the procedure described in Example 3. Another analogous modification will now be set forth in detail.

A portion of Sheet I is first coated lightly with a 2% solution of phenanthrene quinone in acetone. The dried sheet is first exposed through a negative transparency. 55 For this purpose a photographic plate having transparent image areas on a black background, obtained by photographing a printed original, may be used; or a transparency as provided in Example 9 may be substituted. Exposure is to light from the tungsten filament source of Example 2 for a period of 20 seconds, i.e., sufficient to convert essentially all of the quinone to a reductant at the light-struck areas. The sheet is then heated for 10 seconds at 130° C., forming a transposed copy having a brown image on a faint yellow background. The sheet is 60 placed in face-to-face contact with a second portion of Sheet I and the composite is heated for 10 seconds at 130° C. The visibly unchanged second sheet is then exposed to the light source for 20 seconds and heated for 10 seconds at 130° C. to produce a retransposed copy having white images on a brownish background.

What is claimed is as follows:

1. A copysheet product adapted for forming a transposed copy of a graphic original on exposure to actinic radiation applied in a pattern corresponding to said original followed by moderate heating, said copysheet in-

cluding an initially heat-resistant light-activatable layer comprising a water-insoluble light-stable silver salt and a photosensitive progenitor of a silver reducing agent, said progenitor being characterized as causing the precipitation of silver from a normally stable dilute solution containing reactable quantities of said progenitor and silver ion on exposure of said solution to radiation from a B-H 6 lamp at a distance of 9 inches for three minutes.

2. A copysheet product adapted for forming a transposed copy of a transparency on exposure to actinic radiation applied through said transparency followed by moderate heating, said copysheet comprising a backing and an initially heat-resistant light-activatable layer comprising a water-insoluble light-stable silver salt and a photosensitive diazo progenitor of a silver reducing agent, said progenitor being characterized as causing the precipitation of silver from a normally stable dilute solution containing reactable quantities of said progenitor and silver ion on exposure of said solution to radiation from a B-H 6 lamp at a distance of 9 inches for three minutes.

3. A copysheet product adapted for forming a transposed copy of a transparency on exposure to actinic radiation applied through said transparency followed by moderate heating, said copysheet comprising a visibly opaque paper-like backing having an initially heat-resistant light-activatable layer comprising a water-insoluble light-stable silver salt and a photosensitive diazo progenitor of a silver reducing agent, said progenitor being characterized as causing the precipitation of silver from a normally stable dilute solution containing reactable quantities of said progenitor and silver ion on exposure of said solution to radiation from a B-H 6 lamp at a distance of 9 inches for three minutes.

4. A copysheet product adapted for forming a transposed copy of a transparency on exposure to actinic radiation applied through said transparency followed by moderate heating, said copysheet comprising a transparent backing having a transparent initially heat-resistant light-activatable layer comprising a water-insoluble light-stable silver salt and a photosensitive diazo progenitor of a silver reducing agent, said progenitor being characterized as causing the precipitation of silver from a normally stable dilute solution containing reactable quantities of said progenitor and silver ion on exposure of said solution to radiation from a B-H 6 lamp at a distance of 9 inches for three minutes.

5. A copysheet product comprising a backing and an initially heat-resistant light-activatable layer comprising a water-insoluble light-stable blend of a silver soap and a fatty acid, a toner for the silver image, and a photosensitive progenitor of a silver reducing agent, said progenitor being characterized as causing the precipitation of silver from a normally stable dilute solution containing reactable quantities of said progenitor and silver ion on exposure of said solution to radiation from a B-H 6 lamp at a distance of 9 inches for three minutes and said layer including a light-stable tertiary alkyl phenol mild reducing agent for silver in an amount sufficient to cause slow partial reduction of said silver soap with moderate darkening of said sheet at moderately elevated temperature.

6. A copysheet product comprising a transparent backing and a transparent initially heat-resistant light-activatable layer comprising finely divided water-insoluble silver soap of long-chain fatty acid, a toner for the silver image, and a photosensitive progenitor of a silver reducing agent, said progenitor being characterized as causing the precipitation of silver from a normally stable dilute solution containing reactable quantities of said progenitor and silver ion on exposure of said solution to radiation from a B-H 6 lamp at a distance of 9 inches for three minutes.

7. A copysheet comprising a backing and an initially heat-resistant light-activatable layer comprising a film-forming polymeric binder, a water-insoluble silver soap of a long-chain fatty acid, a toner for the silver image, and

a photosensitive diazo progenitor of a silver reducing agent, said progenitor being characterized as causing the precipitation of silver from a normally stable dilute solution containing reactable quantities of said progenitor and silver ion on exposure of said solution to radiation from a B-H 6 lamp at a distance of 9 inches for three minutes.

8. The copysheet of claim 7 in which the diazo compound is a dialkylaminobenzenediazonium hexafluorophosphate.

9. The copysheet of claim 7 in which the diazo compound is a dialkylaminobenzenediazonium tetrafluoroborate.

10. A copysheet comprising a backing having an initially heat-resistant light-activatable layer comprising a water-insoluble light-stable silver salt, a photosensitive progenitor of a silver reducing agent, said progenitor being characterized as causing the precipitation of silver from a normally stable dilute solution containing reactable quantities of said progenitor and silver ion on exposure of said solution to radiation from a B-H 6 lamp at a distance of 9 inches for three minutes, and a photoreducible dye.

11. The copysheet of claim 1 wherein the progenitor is volatilizable from said coating at about 100-150° C.

12. A photosensitive transfer sheet capable after being exposed to actinic radiation of causing the reduction of water-insoluble silver soap on heating in contact therewith and comprising a backing and a reactant layer including as the sole chemically reactive component a photosensitive progenitor of a volatilizable silver reducing agent, said progenitor being characterized as causing the precipitation of silver from a normally stable dilute solution containing reactable quantities of said progenitor and silver ion on exposure of said solution to radiation from a B-H 6 lamp at a distance of 9 inches for three minutes.

13. The transfer sheet of claim 12 in which the photosensitive silver reductant progenitor is a diazo compound.

14. The transfer sheet of claim 13 in which the photosensitive silver reductant progenitor is an alkali metal hydroxybenzenediazosulfonate.

15. The transfer sheet of claim 13 in which the photosensitive silver reductant progenitor is a dialkylaminobenzenediazonium salt.

16. The method of making a transposed print of a graphic original comprising exposing to a differential pattern of actinic radiation corresponding to said original a sheet material having a photosensitive layer including a photosensitive progenitor of a silver reducing agent, said progenitor being characterized as causing the precipitation of silver from a normally stable dilute solution containing reactable quantities of said progenitor and silver ion on exposure of said solution to radiation from a B-H 6 lamp at a distance of 9 inches for three minutes, and then heating said layer while in inter-reactive association with a corresponding layer of a water-insoluble light-stable silver salt and a silver image toner.

17. The method of making a transposed print of a transparency comprising exposing to actinic radiation through said transparency a copysheet having an initially heat-resistant light-activatable layer including a water-insoluble light-stable silver salt, a silver image toner, and a photosensitive progenitor of a silver reducing agent, and heating said sheet to render visibly distinct the light-struck areas thereof; said progenitor being characterized as causing the precipitation of silver from a normally stable dilute solution containing reactable quantities of said progenitor and silver ion on exposure of said solution to radiation from a B-H 6 lamp at a distance of 9 inches for three minutes.

18. The method of making a transposed print of a transparency comprising exposing to actinic radiation in a pattern determined by said transparency a transfer sheet having a surface layer including a photosensitive progenitor of a silver reducing agent, said progenitor being characterized as causing the precipitation of silver from a

normally stable dilute solution containing reactable quantities of said progenitor and silver ion on exposure of said solution to radiation from a B-H 6 lamp at a distance of 9 inches for three minutes, placing the thus exposed transfer sheet in face-to-face contact with a print sheet having a surface layer including a water-insoluble light-stable silver salt and a silver image toner, and heating the composite to an extent sufficient to cause formation of silver image on said print sheet at areas corresponding to the irradiated areas of said transfer sheet.

19. The method comprising exposing to a differential pattern of actinic radiation a sheet material including an initially heat-resistant light-activatable layer comprising a water-insoluble light-stable silver salt and a photosensitive progenitor of a silver reducing agent, said progenitor being characterized as causing the precipitation of silver from a normally stable dilute solution containing reactable quantities of said progenitor and silver ion on exposure of said solution to radiation from a B-H 6 lamp at a distance of 9 inches for three minutes; heating said

sheet to render visibly distinct the light-struck areas thereof; converting the remaining progenitor to silver reductant by further exposure to actinic radiation and in a pattern corresponding to the initially unreacted areas; and reacting said reductant in said pattern with a silver salt layer of a copysheet by heating in contact therewith.

#### References Cited

##### UNITED STATES PATENTS

|    |           |         |               |          |
|----|-----------|---------|---------------|----------|
| 10 | 2,066,918 | 1/1937  | Poser et al.  | 96—49    |
|    | 2,067,690 | 1/1937  | Alink et al.  | 96—49    |
|    | 2,183,447 | 12/1939 | Dippel et al. | 96—49    |
|    | 3,094,619 | 6/1963  | Grant         | 117—36.8 |
| 15 | 3,107,174 | 10/1963 | Wartman       | 117—36.8 |
|    | 3,218,166 | 11/1965 | Reitter       | 117—36.8 |

NORMAN G. TORCHIN, Primary Examiner.

R. E. FICHTER, Assistant Examiner.